

# UNITED STATES PATENT OFFICE.

LEWIS HERMAN, JR., OF SUMMER HILL, NEW SOUTH WALES, AUSTRALIA.

## MANUFACTURE OF HATS.

1,379,341.

Specification of Letters Patent. Patented May 24, 1921.

No Drawing.

Application filed June 30, 1919. Serial No. 307,847.

To all whom it may concern:

Be it known that I, LEWIS HERMAN, Jr., a subject of the King of Great Britain and Ireland, residing at 43 Smith street, Summer Hill, in the State of New South Wales, Commonwealth of Australia, have invented certain new and useful Improvements in the Manufacture of Hats, of which the following is a specification.

10 The object of this invention is to impart to hats made of woolen or other soft material the "body," resilience and resistance of felt and at the same time render the material completely damp-resistant.

15 To accomplish this purpose I prepare in the manner herein described, a "foundation" designed to lie between the lining and the covering forming the hat material.

I make a solution consisting of sugar of 20 lead, alum, and water, in or about the proportion of two (2), one (1) and ten (10) respectively, and in this I immerse a piece of cotton fabric, preferably flannelette 36 inches in length and 30 inches in width. After 25 the material has been thoroughly soaked it is hung up so as to drain off slowly the surplus moisture and allowed to become thoroughly dry. I then immerse it in a second solution consisting of from one (1) ounce 30 to two and a half (2½) ounces of shellac dissolved in from a half (½) pint to two and a half (2½) pints of wood-spirit or some other solvent spirit and again allow the material to become thoroughly dry.

35 The necessity for allowing so wide a margin in the quantities of the materials composing the second solution arises first from the fact that there will be considerable difference in the weights and qualities of the

40 fabric to be treated and secondly that widely divergent degrees of rigidity will need to be obtained in accordance with the different class of hats in which the material will be used. The one constant condition is that the

45 solution should be sufficient to thoroughly impregnate and moisten the whole of the fabric but not sufficient to allow of any of the solution to drip away when lifted from the soaking vat. It is also of prime im-

50 portance that the fabric when drying should be placed on a horizontal screen, as if hung out in a vertical position the solution would gravitate toward the lower edge with the result of a final inequality in the distribution 55 of the shellac.

If it is desired to produce a "kind" as

distinguished from a "tinny" feel to the material, in other words to increase its flexibility, I add ninety (90) minims of vegetable oil to the second solution. It would be possible to mix the whole of the ingredients of the two solutions and subject the fabric to a single impregnation but I have found the result unsatisfactory.

When this process has been completed the material will have become absolutely damp-resistant and will have acquired a sufficient degree of rigidity to impart to the hat, of which it becomes the "foundation," the required resilience and "body."

I am aware that many stiffening materials have been used for this purpose but none of them being entirely damp-proof, once the hat in which they are used gets wet, it becomes soft and flaccid and loses the resiliency which causes it to regain and retain its shape and "set."

In making up the hat material my "foundation" may be secured between the lining and covering either by quilting or dry 80 heating and blocking or by any of the ordinary trade processes.

In the event of a hat being quilted the needle perforations in all known productions admit the damp, but foundation material manufacture by my method contains a plastic element which under any blocking process will fill up the needle perforations and maintain the water-proof characteristic of the foundation.

I do not confine myself absolutely to the quantities or proportions of the materials used in forming my solutions but those specified I have found after experiments to give the best results. It is possible also that certain chemical equivalents may be found to give similar results. It may be found advisable under certain circumstances to pass the foundation material between rollers for the purpose of more evenly distributing the elastic material formed by the second solution when dry or partially dried out.

By means of this method of treatment I am enabled to produce a "foundation" material which will impart to a hat formed of tweed or other relatively inexpensive materials all the quantities of an expensive felt.

It is obvious also that my "foundation" material may be found highly suitable for other purposes besides the manufacture of hats as it will doubtless provide a cheap and efficient stiffening for men's coats and por-

tions of women's dresses, and also for boot linings, but its principal use will be for the purpose set forth.

What I claim and desire to secure by

5 Letters Patent is:—

1. In the manufacture of hats, a foundation material consisting of a fabric, treated in sequence with a solution of sugar of lead, alum and water, and of shellac and wood

10 spirit.

2. In the manufacture of hats the method of preparing a foundation material consisting in treating a fabric, first with a solution of sugar of lead, alum and water, and subsequently with another of wood spirit **15** and shellac.

Signed at Sydney, N. S. W., this second day of June, 1919.

LEWIS HERMAN, JR.